

# UNITED STATES PATENT OFFICE.

WILLOUGHBY SMITH, OF WHARF ROAD, CITY ROAD, COUNTY OF MIDDLE-  
SEX, ENGLAND.

INSULATING ELECTRICAL CONDUCTORS AND A NEW COMPOUND SUITABLE TO BE USED FOR THIS AND  
OTHER PURPOSES.

**SPECIFICATION** forming part of Letters Patent No. 276,916, dated May 1, 1883.

Application filed March 19, 1883. (No specimens.) Patented in England December 28, 1882, No. 6,196.

*To all whom it may concern:*

Be it known that I, WILLOUGHBY SMITH, a subject of the Queen of Great Britain, residing at Wharf Road, City Road, in the county of Middlesex, England, have invented certain new and useful Improvements in Insulating Electrical Conductors and a new Compound Suited to be Used for this and other Purposes, (for which I have received Letters Patent in Great Britain, No. 6,196, dated December 28, 1882,) of which the following is a specification.

This invention has for its object improvements in insulating electrical conductors and a new compound suited to be used for this and other purposes.

In insulating electrical conductors I take, by preference, gutta-percha of the cheaper sort, such as cannot be used alone in the ordinary process of covering wires, and I mix the gutta-percha with finely-powdered bituminous coal. The coal, which should be of good quality, is ground and sifted through sieves, as flour is prepared. The admixture is made while the gutta-percha is being masticated in the ordinary way in a masticating-machine, or by the use of rollers; or by other means the mixture may be brought about. The proportions may be varied, if the object be simply to improve the working of the composition through the covering-die. This object will be fully attained by the addition of one part, by weight, of ground coal to from ten to five of gutta-percha; but with the object of increasing the bulk of the compound, and to attain the maximum utility

at a given cost, the ground coal may be used 35 in the proportion of one part to two or three of gutta-percha, or even a larger proportion of ground coal may be employed.

The compound is applied to cover the wire or strand, serving as the conductor, by pressing 40 the compound out from a die, through which the wire or strand is also led. The compound is maintained in a plastic condition by heat, and the process is conducted in the same way as at present when covering wires or strands 45 with gutta-percha.

By means of this invention electrical conductors may be well insulated at a much smaller cost than at present.

My compound of gutta-percha and ground 50 coal can also advantageously be used to make battery-cells and like articles. It may be rolled into sheets and used as a substitute for vulcanite. For these purposes a compound consisting of one part of ground coal to three 55 parts of gutta-percha is very suitable.

What I claim is—

1. Insulating electrical conductors by covering them, through a die, with a compound of gutta-percha and ground coal. 60
2. My new plastic insulating compound, consisting of gutta-percha and ground coal intimately mixed.

WILLOUGHBY SMITH.

Witnesses:

JOHN DEAN,

J. WATT,

Both of 17 Gracechurch Street, London.